

Aug. 20, 1940.

A. BROSSETTE

2,212,433

COLLAPSIBLE TUBE

Filed Oct. 5, 1937



A. Brossette, inventor  
by Glascock Downing & Sebold, Atty.

## UNITED STATES PATENT OFFICE

2,212,433

## COLLAPSIBLE TUBE

Alois Brossette, Solingen, Germany

Application October 5, 1937, Serial No. 167,437  
In Germany July 2, 1936

15 Claims. (Cl. 93—94)

My invention relates to a collapsible tube such as is ordinarily used as a container of plasti-  
5 cal, liquid or pulverized materials, e. g. for cos-  
metical purposes, and is particularly concerned  
with improvements in the structure of the tube  
and in the process of manufacturing it.

An object of my invention is to produce such  
tubes of an organic cellulose-containing sheet  
material, particularly of a transparent sheet  
10 of cellulose derivatives. Another object is an  
improved process of manufacture resulting in a  
tube of an organic material which is not inferior  
to, and may compete with tubes of sheet metal  
and satisfies all reasonable requirements.

15 My invention is based on the fact that, in any  
tube produced by winding up a strip of organic  
sheet material and by gluing the superimposed  
plies together by an intermediate layer of bind-  
ing material, the intermediate layer has a func-  
20 tion which has not been recognized prior to my  
invention. I have found that the nature of the  
intermediate layer is controlling on the qualities  
of the product. Moreover I have found it neces-  
25 sary to subject the sheet of a cellulose material  
to a preparatory treatment thus enabling the  
sheet to properly cooperate with the intermedia-  
te layer. The primary consideration for the  
choice of the intermediate layer is the necessity  
30 that such layer should not only act as a glue but  
should also have additional functions, particu-  
larly the function as an insulating medium ren-  
dering the tube moisture-proof.

I have found that the tubes produced in ac-  
cordance with my invention are entirely free  
35 from the shortcomings of the tubes of a cellu-  
lose material produced in accordance with known  
processes.

The improved process comprises preferably  
40 three steps, to-wit coating the cellulose sheet  
material with a moisture-proof layer, coating  
such layer with a gum or glue and winding up  
the sheet material so treated to form a cylind-  
rical body from which the collapsible tube is  
45 produced in a known manner.

For the purpose of my invention I prefer to  
use a sheet material consisting of a cellulose  
ester such as acetyl cellulose or nitro-cellulose.  
I may also use other cellulose derivatives such  
50 as viscose. Such sheet materials or foils are  
available on the market. Very frequently they  
are coated with a varnish comprising a solution  
of nitro-cellulose or cellulose or the like.

Further objects of my invention will appear  
from the description of a preferred embodiment  
55 thereof following hereinafter with reference to

the drawing in which I have shown a tube which  
may be manufactured by my improved process.

The tube shown on the drawing comprises the  
cylindrical body A consisting of superimposed  
plies formed by winding up a strip of sheet ma-  
5 terial on a mandrel, the plies being glued to-  
gether so as to constitute a pliable sleeve. The  
lower end of the tube thus formed is closed in  
any suitable manner, e. g. by pressing the op-  
posed walls of the tube upon each other and by 10  
folding them over, as indicated at B. The upper  
end C is pressed in suitable dies to form a mouth  
piece provided with threads D to receive a  
threaded cover, not shown.

My invention is primarily concerned with the 15  
first step of this process, i. e. the winding of the  
strip of material upon a mandrel to form the  
tube body A.

In producing this body I may start with a strip  
of acetyl cellulose and with a liquid produced 20  
by mixing collodium elasticum, traumaticin and  
benzyl alcohol. Traumaticin is a solution of  
gutta-percha in a solvent comprising trichlorae-  
thylen and an acetone-like medium such as  
drawin which is adapted to partly dissolve acetyl 25  
cellulose. Drawin is an acetone solution which  
is mixed with cheaper solvents. This liquid is  
applied to one or both sides of the sheet material  
in a thin layer, e. g. by means of rollers. The  
liquid has the effect of superficially dissolving the 30  
sheet material thus rendering the surface there-  
of porous whereby the gutta-percha contained  
in the liquid is enabled to penetrate into the  
pores. Then the solvent is removed, e. g. vapor-  
35 ized in vacuum. As a result, the gutta-percha  
will constitute a thin coat which is intimately  
interlocked with the sheet material. The col-  
lodium elasticum contained in the liquid will  
40 form a film of nitro-cellulose. The benzyl al-  
cohol serves solely the function of producing a  
mixture between traumaticin and collodium  
elasticum and disappears when the solvent is  
vaporized. After the vaporization, the sheet ma-  
45 terial of acetyl cellulose is coated and intimately  
interlocked with a layer of gutta-percha consti-  
tuting a moisture-proof material. This layer of  
gutta-percha is coated in its turn with a layer  
50 of a nitro-cellulose varnish. The coated sheet  
material so produced is now in a condition to be  
provided on its coated face with a layer of a  
suitable adhesive of glue, containing e. g. a  
polymerization product, such as polyacrylacid-  
55 ester or gutta-percha. I prefer to dissolve this  
adhesive in a volatile solvent containing a small  
percentage of a liquid adapted to superficially

5

10

15

20

25

30

35

40

45

50

55

dissolve the layer of varnish. Suitable solvents are, for instance, chloroform, sulfuric or ethylic ether, acetone, gasoline, benzol or benzene, alcohol and the like. Therefore, when the adhesive 5 is applied to the coated sheet material, the coating of varnish thereon will be superficially dissolved and rendered porous enabling the adhesive to penetrate into the pores of the layer of varnish.

Before the adhesive layer is dried, the sheet 10 material is wound up on a suitable mandrel. In this operation the adhesive on one ply will contact with the cellulose material of the superimposed ply and will superficially dissolve the cellulose material thereof. As a result, the adhesive 15 will intimately interlock with the superimposed layer of cellulose material and will thus bind the two plies effectively one to another.

I may admix a pigment either to the liquid 20 consisting of collodium elasticum, traumaticin and benzyl alcohol or to the adhesive, if it is desired to produce an opaque tube. Such a pigment may be a pulverized aluminum or a suitable color. The admixture of a pulverized aluminum 25 has the additional advantage of enhancing the resistivity against moisture.

In another form of my improved process the first step comprises superficially dissolving the sheet material of acetyl cellulose, e. g. by use of a suitable solvent such as acetone. Then a 30 solution of gutta-percha is applied to the sheet material to produce the moisture-proof layer. This layer is dried and is then coated with a suitable varnish. After the coat of varnish has been dried, it is superficially dissolved again and 35 then provided with a coat of adhesive. Before the adhesive is dry, the sheet material is wound up upon the mandrel and is then permitted to dry.

Also the layer of pigment may be added in a 40 separate step.

The cellulose sheet material in its commercial form is usually coated with a layer of varnish which is easier soluble in the solvents mentioned above than the cellulose material and is therefore particularly adapted to intimately bind the moisture-proof layer to the sheet material.

While I have described two preferred embodiments of my invention, I wish it to be clearly understood that my invention is capable of numerous modifications within the scope of the 50 appended claims.

Thus I may use other moisture-proof materials than gutta-percha to coat the sheet material, e. g. rubber. Also, other cellulose-containing 55 sheet materials than transparent sheets may be used, e. g. paper. Moreover anyone skilled in the art will readily appreciate that a great multiplicity of various solvents may be selected depending on the properties of the sheet material, of the moisture-proof coat and of the adhesive.

What I claim is:

1. Process for the production of tubes for the reception of plastic materials consisting in treating a sheet of a transparent cellulose derivative 60 with a solution of collodium elasticum, traumaticin and benzyl alcohol, coating said treated sheet with a material substantially different from and with superficial solvent properties for the cellulose derivative material, said coating serving as an intermediate layer having adhesive, isolating 65 and insulating properties and winding said sheet onto a cylinder to form a tube, said coating holding the wound sheet together.

2. Process for the production of tubes for the 70 reception of plastic materials consisting in coating a sheet of a transparent cellulose derivative

with a varnish, treating said sheet with a solution of collodium elasticum, traumaticin and benzyl alcohol, coating said treated sheet with a material substantially different from, and with superficial solvent properties for, the cellulose derivative material, said coating serving as an intermediate layer having adhesive, isolating and insulating properties winding the sheet onto a cylinder to form a tube, said adhesive coating holding the wound sheet together. 10

3. Process for the production of tubes for the reception of plastic materials consisting in treating a sheet of a transparent cellulose derivative with a solution of collodium elasticum, traumaticin and benzyl alcohol, coating said treated sheet 15 with a material substantially different from, and with superficial solvent properties for, the cellulose derivative material, said coating containing a pigment carrier and serving as an intermediate layer having adhesive, isolating and insulating properties, winding the sheet onto a cylinder to form a tube, said adhesive coating holding the wound sheet together. 20

4. A process for the production of tubes for the reception of plastic materials consisting in coating a sheet of a transparent cellulose derivative with a varnish, treating said sheet with a solution of collodium elasticum, traumaticin and benzyl alcohol, coating said treated sheet with a material substantially different from, and with superficial 30 solvent properties for, the cellulose derivative material, said coating containing a pigment carrier, and serving as an intermediate layer having adhesive, isolating and insulating properties, winding the sheet onto a cylinder to form a tube, said adhesive coating holding the wound sheet together. 35

5. A process for the production of tubes for the reception of plastic materials consisting in treating a sheet of a transparent cellulose derivative with a solution of collodium elasticum, traumaticin and benzyl alcohol, coating said treated sheet with a material substantially different from, and with superficial solvent properties for, the cellulose derivative material, said coating containing aluminium powder and serving as an intermediate layer having adhesive, isolating and insulating properties, winding the sheet onto a cylinder to form a tube, said coating holding the wound sheet together. 40

6. A process for the production of tubes for the reception of plastic material consisting in coating a sheet of a transparent cellulose derivative with a varnish, treating said sheet with a solution of collodium elasticum, traumaticin and benzyl alcohol, coating said treated sheet with a material substantially different from, and with superficial solvent properties for, the cellulose derivative material, said coating containing aluminium powder and serving as an intermediate 55 layer having adhesive, isolating and insulating properties, winding said sheet onto a cylinder to form a tube, said adhesive coating holding the wound sheet together.

7. In a process for the production of tubes for the reception of plastic materials, the steps which comprise treating a sheet of a cellulose derivative with a moisture-proof material which is dissolved in a liquid having a solvent action with respect to the cellulose derivative, coating said 70 treated sheet with an adhesive with superficial solvent properties for the treated cellulose derivative sheet, and winding said sheet onto a mandrel to form a tube the walls of which consist of a plurality of superimposed layers of said 75

wound sheet with intermediate layers of said moisture-proof material and said adhesive between the said superimposed layers.

8. In a process for the production of tubes for the reception of plastic materials, the steps which comprise treating a sheet of a cellulose derivative with a moisture-proof material of the group comprising gutta-percha and rubber which is dissolved in a liquid having a solvent action with respect to the cellulose derivative, coating said treated sheet with an adhesive with superficial solvent properties for the treated cellulose derivative sheet, and winding said sheet onto a mandrel to form a tube the walls of which consist of a plurality of superimposed layers of said wound sheet with intermediate layers of said moisture-proof material and said adhesive between the said superimposed layers.

9. In a process for the production of tubes for the reception of plastic materials, the steps which comprise treating a sheet of a cellulose derivative with a moisture-proof material which is dissolved in a liquid having a solvent action with respect to the cellulose derivative, coating said treated sheet with an adhesive with superficial solvent properties for the treated cellulose derivative sheet, of the group comprising solutions of polymerisation products and gutta-percha, and winding said sheet onto a mandrel to form a tube the walls of which consist of a plurality of superimposed layers of said wound sheet with intermediate layers of said moisture-proof material and said adhesive between the said superimposed layers.

10. In a process for the production of tubes for the reception of plastic materials, the steps which comprise treating a sheet of a cellulose derivative with a moisture-proof material which is dissolved in a liquid having a solvent action with respect to the cellulose derivative, coating said treated sheet with polyacrylacidester dissolved in a volatile solvent containing a small percentage of a liquid adapted to dissolve the surface of the treated cellulose derivative sheet, and winding said sheet onto a mandrel to form a tube the walls of which consist of a plurality of superimposed layers of said wound sheet with intermediate layers of said moisture-proof material and said polyacrylacidester between the said superimposed layers.

11. In a process for the production of tubes for the reception of plastic materials, the steps which comprise treating a sheet of a cellulose derivative with a moisture-proof material of the group comprising gutta-percha and rubber which is dissolved in a liquid having a solvent action with respect to the cellulose derivative, coating said treated sheet with an adhesive with superficial solvent properties for the treated cellulose derivative sheet, of the group comprising solutions of polymerisation products and gutta-percha, and winding said sheet onto a mandrel to form a tube the walls of which consist of a plurality of superimposed layers of said wound sheet with intermediate layers of said moisture-proof material and said adhesive between the said superimposed layers.

12. In a process for the production of tubes for the reception of plastic materials, the steps which comprise treating a sheet of a cellulose derivative with a moisture-proof material which is dissolved in a liquid having a solvent action with respect to the cellulose derivative, coating said treated sheet with an adhesive with superficial solvent properties for the treated cellulose derivative sheet, and winding said sheet onto a mandrel before said adhesive layer is dried, to form a tube the walls of which consist of a plurality of superimposed layers of said wound sheet with intermediate layers of said moisture-proof material and said adhesive between the said superimposed layers.

13. In a process for the production of tubes for the reception of plastic materials, the steps which comprise superficially dissolving a sheet of a cellulose derivative, treating said sheet with a moisture-proof material which is dissolved in a liquid having a solvent action with respect to the cellulose derivative, coating said treated sheet with an adhesive with superficial solvent properties for the treated cellulose derivative sheet, and winding said sheet onto a mandrel to form a tube the walls of which consist of a plurality of superimposed layers of said wound sheet with intermediate layers of said moisture-proof material and said adhesive between the said superimposed layers.

14. In a process for the production of tubes for the reception of plastic materials, the steps which comprise superficially dissolving a sheet of a cellulose derivative, treating said sheet with a moisture-proof material which is dissolved in a liquid having a solvent action with respect to the cellulose derivative, drying and coating the treated sheet with a varnish, drying said varnish coating, superficially redissolving the varnish coating and coating said treated sheet with an adhesive with superficial solvent properties for the treated cellulose derivative sheet, and winding said sheet onto a mandrel to form a tube the walls of which consist of a plurality of superimposed layers of said wound sheet with intermediate layers of said moisture-proof material and said adhesive between the said superimposed layers.

15. In a process of producing tubes for the reception of plastic material from commercial cellulose sheet material having a varnish coating on its surface, the steps which comprise treating a sheet of a cellulose derivative with a moisture-proof material which is dissolved in a liquid having a solvent action with respect to the said varnish coating, coating said treated sheet with an adhesive with superficial solvent properties for the treated cellulose derivative sheet, and winding said sheet onto a mandrel to form a tube the walls of which consist of a plurality of superimposed layers of said wound sheet with intermediate layers of said moisture-proof material and said adhesive between the said superimposed layers.

ALOIS BROSSETTE. 65